# EUROPEAN PATENT SPECIFICATION

(11) **EP 3 395 988 B1**
(45) Date of publication and mention of the grant of the patent: **07.02.2024**
(21) Application number: 16879310.7
(22) Date of filing: 21.12.2016
(51) Int. Cl.: C22C 38/02, C22C 38/04, C22C 38/08, C22C 38/12, C22C 38/14, C22C 38/16, C22C 38/06, C22C 38/00, C21D 8/02, C21D 9/46

(54) **HIGH-STRENGTH STRUCTURAL STEEL SHEET EXCELLENT IN HOT RESISTANCE AND MANUFACTURING METHOD THEREOF**
HOCHFESTES BAUSTAHLBLECH MIT HERVORRAGENDER HITZEBESTÄNDIGKEIT UND HERSTELLUNGSVERFAHREN DAFÜR
TÔLE D'ACIER STRUCTURAL HAUTE RÉSISTANCE PRÉSENTANT UNE EXCELLENTE RÉSISTANCE À CHAUD ET SON PROCÉDÉ DE FABRICATION

(30) Priority: 23.12.2015 KR 20150184775
(43) Date of publication of application: 31.10.2018
(73) Proprietor: POSCO Co., Ltd, Pohang-si, Gyeongsangbuk-do 37859 (KR)
(72) Inventor: KIM, Woo-Gyeom, Pohang-si, Gyeongsangbuk-do 37877 (KR); KIM, Han-Kyu, Pohang-si, Gyeongsangbuk-do 37877 (KR); KIM, Sang-Ho, Pohang-si, Gyeongsangbuk-do 37877 (KR)
(74) Representative: Potter Clarkson
(86) International application number: PCT/KR2016/014964
(87) International publication number: WO 2017/111443

(56) References cited:
- EP-A2- 2 660 346
- WO-A1-2009/082156
- JP-A- H11 152 540
- JP-A- S63 183 123
- JP-A- 2007 056 348
- JP-A- 2007 056 348
- JP-A- 2010 121 149
- JP-A- 2010 121 149
- KR-A- 20030 053 767
- KR-A- 20110 022 308

## Description

### [Technical Field]

The present invention relates to a high-strength structural steel sheet having excellent heat treatment resistance and a manufacturing method thereof.

### [Background Art]

The exteriors of ships and marine and architectural structures have both planar and curved surfaces.

Since planar processing is determined during a plate material forming process, the exterior is formed without performing a separate process when ships or marine structures are constructed, but in the case of a curved surface forming process, a plate material is processed. In order to perform this process, linear heating, an operation of heating a surface of steel sheet, is performed.

Bending work, based on linear heating, utilizes properties in which a heated portion is deformed due to constraint from a non-heated region around the heated portion when the heated portion contracts due to cooling after being heat-expanded.

In order to apply such linear heating, a surface of the steel sheet is heated to a temperature of about 600 to 900°C or water-cooled after heating, and thus, after the linear heating, physical properties of the steel sheet may be lowered. When a steel material is heated to an austenite start transformation temperature, if the steel material is heated to above the transformation temperature or a recrystallization temperature due to annealing of dislocations, or the like, the material is mainly deteriorated due to the growth of a crystal grain.

Further, the steel sheet may be embrittled due to a heat cycle of heating and cooling of the surface of the steel sheet, resulting in deterioration of toughness.

Therefore, development of a high-strength structural steel sheet having excellent heat treatment resistance, which has excellent yield strength, tensile strength, and impact toughness even after linear heating, and a manufacturing method thereof are required.

Publication no. EP 2660346 A2 discloses a high-strength steel sheet having superior toughness at cryogenic temperature and a tensile strength of 490 MPa or more through controlling the contents of Mn, Si, Al and Sb and through a microstructure comprising, in area percentage, 99% or more of acicular ferrite and 1% or less of austenite/martensite (MA).

### [Disclosure]

### [Technical Problem]

An aspect of the present invention is to provide a high-strength structural steel sheet having excellent heat treatment resistance, which has excellent yield strength, tensile strength, and impact toughness, even after linear heating, and a manufacturing method thereof are required.

### [Technical Solution]

According to an aspect of the present invention a high-strength structural steel sheet having excellent heat treatment resistance includes: by weight percent (wt%), 0.03 to 0.07% of C, 0.05 to 0.2% of Si, 1.6 to 2.3% of Mn, 0.008% or less of P, 0.002% or less of S, 0.025% or less of Al, 0.1 to 0.4% of Cu, 1.4 to 2.3% of Ni, 0.08 to 0.2% of Mo, 0.01 to 0.025% of Nb, 0.008 to 0.02% of Ti, 0.001 to 0.008% of N, the remainder being Fe, and unavoidable impurities, wherein, by volume percent (vol%), a microstructure within 10 mm of the surface consists of 20% or less of polygonal ferrite and 80% or more of acicular ferrite, and wherein the steel sheet has a yield strength of 500 MPa or greater, tensile strength of 600 MPa or greater, and impact toughness of 100 J or greater at -40°C.

According to an aspect of the present invention, a method of manufacturing a high-strength structural steel sheet having excellent heat treatment resistance includes: reheating a slab at 1100 to 1200°C wherein the slab includes, by weight percent (wt%), 0.03 to 0.07% of C, 0.05 to 0.2% of Si, 1.6 to 2.3% of Mn, 0.008% or less of P, 0.002% or less of S, 0.025% or less of Al, 0.1 to 0.4% of Cu, 1.4 to 2.3% of Ni, 0.08 to 0.2% of Mo, 0.01 to 0.025% of Nb, 0.008 to 0.02% of Ti, 0.001 to 0.008% of N, the remainder being Fe, and unavoidable impurities; performing non-recrystallization region rolling on the reheated slab at 750 to 850°C; and performing cooling to a cooling end temperature of 380 to 440°C at a cooling rate of 10°C/sec. or faster after the non-recrystallization region rolling, wherein the steel sheet has a yield strength of 500 MPa or greater, tensile strength of 600 MPa or greater, and impact toughness of 100 J or greater at -40°C.

The invention is defined in the appended claims.

The foregoing technical solutions do not fully enumerate all of the features of the present invention. The foregoing and other objects, features, aspects and advantages of the present invention will become more apparent from the following detailed description of the present invention when taken in conjunction with the accompanying drawings.

### [Advantageous Effects]

As set forth above, according to an exemplary embodiment in the present invention, the high-strength structural steel sheet, which has excellent yield strength, tensile strength, and low-temperature impact toughness even after linear heating by having excellent heat treatment resistance, as well as before the linear heating, and a manufacturing method thereof may be provided.

### [Description of Drawings]

FIG. 1 is a schematic view illustrating an example of curved surface forming by linear heating.
FIG. 2 is a photograph of a cross-sectional structure of a steel sheet of Inventive Example 1 at a depth of 10 mm from a surface thereof.

### [Best Mode for invention]

Hereinafter, exemplary embodiments of the present invention will now be described in detail with reference to the accompanying drawings. The exemplary embodiments may, however, be exemplified in many different forms and should not be construed as being limited to the specific exemplary embodiments set forth herein. Also, these exemplary embodiments are provided so that this disclosure will be thorough and complete, and will fully convey the scope of the inventive concept to those skilled in the art.

The inventors of the present disclosure have found that when the high-strength structural steel sheet is linearly heated to be bent to have a curved surface in the appearance of ships, marine structures and building structures, physical properties of the steel sheet may be lowered after the linear heating.

Since the surface of the steel sheet is heated to 600 to 900°C during linear heating, a base structure and a grain boundary are softened, a crystal grain is grown, carbide (Fe₃C) is coarsened, causing a phenomenon in which both strength and toughness are degraded.

Further, the heating to the austenite start transformation temperature causes deterioration of the material due to annealing of dislocations, and the like, and when the steel sheet is heated to above the transformation temperature or above the recrystallization temperature, the material is mainly degraded due to the growth of the crystal grains.

In order to solve the problems, the inventors of the present disclosure have found that when a microstructure within 10 mm or less from a surface consists of, by volume fraction, 80% or more of acicular ferrite and 20% or less of polygonal ferrite through low temperature rolling and strong cooling by lowering an Ar₃ temperature by adding large amounts of Mn and Ni, growth of a crystal grain after linear heating may be prevented and growth of a crystal grain and formation of coarse carbide may be prevented using a grain boundary pinning effect of precipitates of NbC and Mo₂C, whereby, the inventors noticed that, a high-strength structural steel sheet having excellent yield strength, tensile strength, and impact toughness even after linear heating, as well as before the linear heating, and a manufacturing method thereof can be provided, thus completing the present invention.

Hereinafter, the high-strength structural steel sheet having excellent heat treatment resistance according to an aspect of the present invention will be described.

A high-strength structural steel sheet having excellent heat treatment resistance according to an aspect of the present invention is defined in claim 1.

### C: 0.03 to 0.07% by weight % (hereinafter, the unit of each element content is wt%)

C is a very important element for securing strength.

In order to secure sufficient strength, 0.03% or more of C is added. If C is excessively added, a coarse carbide may be formed during cooling after the linear heating to lower impact toughness, and thus, the upper limit of C is 0.07%.

### Si: 0.05 to 0.2%

Si is a useful element as a deoxidizing agent, but if the content of C is excessive, toughness may be lowered. For deoxidation, the Si content is 0.05% or more. However, if the Si content exceeds 0.2%, toughness may be lowered. Therefore, the Si content is 0.05 to 0.2%.

### Mn: 1.6 to 2.3%

Mn has an effect of improving strength as a solid solution strengthening element and improving grain refinement and toughness of a base material. In addition, formation of polygonal ferrite may be minimized by low temperature rolling and strong cooling by lowering the Ar₃ temperature.

In order to sufficiently exhibit the above effect, Mn is added in an amount of 1.6% or more. If, however, Mn is excessively added, a nonmetallic inclusion of MnS is formed at a central portion, and the MnS inclusion may be stretched after rolling to significantly lower low temperature toughness. Therefore, the upper limit thereof is 2.3%.

### P: 0.008% or less

P is an element advantageous for improving strength and corrosion resistance but since it is an element which greatly hinders impact toughness, it is advantageous to keep it as low as possible, and therefore, the upper limit thereof is 0.008%.

### S: 0.002% or less

Since S forms MnS, or the like, to greatly deteriorate impact toughness, it is advantageous to add it as little as possible, so that the upper limit is 0.002%.

### Al: 0.025% or less

Al, an element for effectively performing deoxidation, is preferably controlled to 0.005 to 0.025%. It is not necessary to specifically control a lower limit, but Al may be included by 0.005% or more for deoxidation.

### Cu: 0.1 to 0.4%

Cu, a solid solution strengthening and precipitation strengthening element, is an element capable of improving strength while minimizing a decrease in toughness of the base material. In order to achieve a sufficient strength improvement effect, Cu is contained in an amount of 0.1% or more. Meanwhile, the excessive addition of Cu may cause defects on a surface of the steel due to hot brittleness, so the upper limit thereof is 0.4% or less.

### Ni: 1.4 to 2.3%

Ni is an element capable of simultaneously improving both strength and toughness of a base material. In addition, formation of polygonal ferrite may be minimized by low temperature rolling and strong cooling by lowering the Ar₃ temperature.

If the Ni content is less than 1.4%, the above-mentioned effect is insufficient. If the Ni content is more than 2.3%, curability may be increased and impact toughness may be lowered due to formation of bainite. Therefore, the Ni content is 1.4 to 2.3%.

### Mo: 0.08 to 0.2%

Mo is an element which effectively increases strength by the addition of a small amount, and Mo is added in an amount of 0.08% or more in order to form precipitates of fine Mo-C series after linear heating to prevent deterioration of strength. However, since coarse precipitates may occur due to excessive addition of Mo, the upper limit thereof is 0.2% or less.

### Nb: 0.01 to 0.025%

Nb dissolved in the steel sheet prior to linear heating is precipitated in the form of NbC or NbCN during the linear heating to improve strength of the base material. Nb is important to maintain strength after linear heating, and at least 0.01% must be added in order to effectively demonstrate the addition effect of Nb. However, excessive addition of Nb may coarsen the precipitates, and therefore, the upper limit thereof is 0.025% or less.

### Ti: 0.008 to 0.02%

Ti forms a nitride with N to prevent crystal grains from growing at a high temperature. In order to sufficiently secure such an effect, the Ti content is 0.008% or more. Meanwhile, excessive Ti addition may lower impact toughness due to coarsening of the Ti precipitates, and thus, the upper limit thereof is 0.02%.

### N: 0.001 to 0.008%

N is an element which forms a precipitate together with Ti, Nb and Al to improve strength and toughness by making an austenite structure finer during reheating.

If the N content is less than 0.001%, the above-mentioned effect may not be sufficiently obtained. Meanwhile, when the N content exceeds 0.008%, surface cracking may occur at a high temperature and the residual N may exist in an atomic state to reduce toughness. Therefore, the N content is 0.001 to 0.008%.

The remainder of the steel sheet of the present disclosure is iron (Fe). However, in the ordinary manufacturing process, impurities that are not intended may be inevitably mixed from a raw material or a surrounding environment, so the impurities may not be excluded. These impurities are known to any person skilled in the art of manufacturing, and thus, are not specifically mentioned in this disclosure.

Hereinafter, a microstructure of a high-strength structural steel sheet having excellent heat treatment resistance according to one aspect of the present invention will be described.

According to an aspect of the present invention, a microstructure within 10 mm of the surface of the high-strength structural steel sheet having excellent heat treatment resistance consists of 80% or more of an acicular ferrite and 20% or less of polygonal ferrite, by volume fraction.

Since crystal grains of the polygonal ferrite are easily grown by heating, if the polygonal ferrite is present in an amount of more than 20 volume % in the microstructure within 10 mm, crystal grains may grow, a coarse carbide may be formed, and a base structure may be degraded.

A thickness of the steel sheet is preferably 40 mm or less. If the thickness of the steel sheet exceeds 40 mm, it is difficult to apply bending by linear heating. Here, a minimum thickness of the steel sheet may be 12 mm.

By controlling the alloy composition and microstructure as described above, the steel sheet has yield strength of 500 MPa or greater, tensile strength of 600 MPa or greater, and impact toughness of 100 J or greater at - 40°C. Accordingly, the steel sheet may be preferably used in ships, marine and building structures, and the like.

When the high-strength structural steel sheet having excellent heat treatment resistance having the alloy composition and microstructure as described above is subjected to linear heating, one or more of a Mo₂C precipitate and a NbC precipitate is precipitated.

In an example of curving (bending) by linear heating illustrated in FIG. 1, bending based on linear heating uses properties that a heated portion is deformed by constraint from a surrounding non-heated region when a heated portion contracts due to cooling after thermally expanded.

Also, in the case of linear heating, the surface of the steel sheet is generally heated to 600 to 900°C. Mo dissolved in the steel sheet at a relatively low temperature of 600 to 800°C is precipitated as Mo₂C upon cooling after the linear heating and Nb dissolved in the steel sheet at a relatively high temperature of 800°C or higher is precipitated as NbC upon cooling after the linear heating.

The Mo₂C precipitate or NbC precipitate is precipitated to grain boundaries to inhibit growth of crystal grains (pinning effect) and prevent formation of a coarse carbide. Further, as C is greatly consumed as a precipitate, generation and coarsening of carbide may be prevented. Here, a size of the Mo₂C precipitate and the NbC precipitate is preferably 2 to 20 nm.

Therefore, although the steel sheet according to the present disclosure is linearly heated to 600 to 900°C and subjected to curving, the steel sheet has a yield strength of 500 MPa or greater, tensile strength of 600 MPa or greater, and an impact toughness of 100 J or more at -40°C.

Hereinafter, a method of manufacturing a high-strength structural steel sheet having excellent heat treatment resistance, as another aspect of the present invention, will be described.

The method of manufacturing a high-strength structural steel sheet having excellent heat treatment resistance, as another aspect of the present invention, is defined in claim 3 and includes:
reheating a slab having the above-described alloy composition at 1100 to 1200°C;
performing non-recrystallization region rolling on the reheated slab at 750 to 850°C; and performing cooling to a cooling end temperature of 380 to 440°C at a cooling rate of 10°C/sec. or faster after the non-recrystallization region rolling.

### Reheating

The slab having the above-described alloy composition is reheated. The reheating temperature of the slab is 1100 to 1200°C.

### Non-recrystallization region rolling

The reheated slab is subjected to non-recrystallization region rolling at 750 to 850°C. This is to make crystal grains finer.

In order to make the crystal grains finer, the non-recrystallization rolling must be performed at a lowest temperature right above the Ar₃ temperature. In the present invention, since the Ar₃ temperature is sufficiently low by increasing the content of Mn and Ni, non-recrystallization region rolling is performed at 750°C or higher. If the non-recrystallization region rolling temperature is higher than 850°C, grain refinement is difficult to weaken toughness. Therefore, the upper limit of the non-recrystallization region rolling temperature is 850°C, and a more preferable upper limit is 800°C.

### Cooling

After the non-recrystallization region rolling, the steel sheet is cooled to a cooling end temperature of 380 to 440°C at a cooling rate of 10°C/sec. or faster.

By controlling the cooling step as described above, the microstructure within 10 mm of the surface of the steel sheet consists of at least 80% or more of acicular ferrite and 20% or less of polygonal ferrite by a volume fraction.

When the cooling rate is less than 10°C/sec. or a cooling finish temperature is higher than 440°C, cooling is not sufficiently performed to form a large amount of polygonal ferrite, cause grain growth, and deteriorate the matrix during linear heating.

Meanwhile, linear heating the cooled steel sheet at a temperature of 600 to 900°C to perform bending may be additionally performed.

By the above-mentioned linear heating, it is possible to bend the steel sheet, and since Mo₂C precipitates and NbC precipitates are precipitated upon cooling after the linear heating, grain growth may be inhibited (pinning effect) and formation of coarse carbide may be prevented.

### [Mode for invention]

Hereinafter, the present invention will be described more specifically by way of examples.

Molten steel having the alloy composition as illustrated in Table 1 below were prepared, and thereafter, steel slabs were prepared using continuous casting. Inventive steels A, B, and C are steel sheets satisfying the component range defined in the present invention, and comparative steels D, F, G, and H are steel sheets having a component range which exceeds or falls short of the component range of the present invention. C of comparative steel D is outside the component range of the present invention, Mo of comparative steel E is outside the component range of the present invention, Nb of the comparative steel F is outside the component range of the present invention, and Ni and Mn of comparative steel G are outside the component range of the present invention.

The inventive steels and comparative steels were rolled and cooled under the manufacturing conditions shown in Table 2 to prepare thick steel sheets. Specifically, rolling end temperatures were 780°C and 880°C, and cooling end temperatures were 400°C and 600°C. The manufactured steel sheets were cut into a size available for linear heating, and linear heating for bending was performed under four temperature conditions (600°C, 700°C, 800°C and 900°C).

Table 3 shows mechanical properties of base materials manufactured under the above-mentioned conditions and mechanical properties after linear heating.

Tensile strength of the base material was measured by taking a JIS1B sample from a full thickness of the steel sheets in a direction perpendicular to a rolling direction and performing a tension test at room temperature. As for low temperature toughness of the base material, a sample was taken in a direction perpendicular to a rolling direction from a portion 2mm directly under from a surface portion of the steel sheet to manufacture a V-notch sample, Charpy impact test was performed on the test sample at -40°C three times and an average value is illustrated in Table 3.

In addition, the microstructure within 10 mm of the surface of the steel sheet was observed and a volume fraction of polygonal ferrite is shown in Table 3. A structure other than the polygonal ferrite was acicular ferrite.

**[Table 1]**

| Classific ation | C | Si | Mn | P | S | Al | Ni | Cu | Mo | Nb | Ti | N |
|---|---|---|---|---|---|---|---|---|---|---|---|---|
| Inventive steel A | 0. 04 2 | 0. 08 6 | 1. 95 | 0. 00 55 | 0. 00 15 | 0. 01 1 | 1. 71 | 0. 27 4 | 0. 13 | 0. 01 5 | 0. 01 0 | 0. 00 38 |
| Inventive steel B | 0. 05 4 | 0. 11 6 | 1. 83 | 0. 00 57 | 0. 00 12 | 0. 01 0 | 1. 75 | 0. 24 9 | 0. 12 5 | 0. 02 1 | 0. 01 2 | 0. 00 42 |
| Inventive steel C | 0. 04 5 | 0. 12 3 | 1. 92 | 0. 00 62 | 0. 00 11 | 0. 01 1 | 1. 82 | 0. 25 4 | 0. 11 9 | 0. 01 3 | 0. 01 3 | 0. 00 39 |
| Comparati ve steel D | 0. 12 6 | 0. 12 3 | 1. 88 | 0. 00 61 | 0. 00 12 | 0. 01 0 | 1. 80 | 0. 24 9 | 0. 12 1 | 0. 01 7 | 0. 01 1 | 0. 00 49 |
| Comparati ve steel E | 0. 05 2 | G. 11 8 | 1 . 91 | 0. 00 52 | 0. 00 14 | 0. 01 5 | 1 . 68 | 0. 26 1 | 0. 05 2 | 0. 02 | 0. 01 2 | 0. 00 51 |
| Comparati ve steel F | 0. 04 6 | 0. 12 1 | 1. 89 | 0. 00 75 | 0. 00 13 | 0. 01 2 | 1. 76 | 0. 24 8 | 0. 12 5 | 0. 00 8 | 0. 01 0 | 0. 00 45 |
| Comparati ve steel G | 0. 04 8 | 0. 11 9 | 1. 25 | 0. 00 65 | 0. 00 13 | 0. 01 3 | 0. 65 | 0. 25 3 | 0. 13 2 | 0. 01 8 | 0. 01 2 | 0. 00 42 |

In Table 1, the unit of each element content is wt%.

**[Table 2]**

| Classifi cation | Steel type | FM start tempera ture | FM end tempera ture | Cooling start tempera ture | Cooling finish tempera ture | Cooli ng rate | Linear heating tempera ture |
|---|---|---|---|---|---|---|---|
| Inventiv e example 1 | Inven tive steel A | 795 | 770 | 732 | 432 | 11.3 | 600 |
| | | | | | | | 700 |
| | | | | | | | 800 |
| | | | | | | | 900 |
| Comparat ive example 1 | Inven tive steel A | 885 | 864 | 832 | 412 | 13.2 | 600 |
| | | | | | | | 700 |
| | | | | | | | 800 |
| | | | | | | | 900 |
| Inventiv e example 2 | Inven tive steel B | 789 | 761 | 726 | 408 | 12.5 | 600 |
| | | | | | | | 700 |
| | | | | | | | 800 |
| | | | | | | | 900 |
| Comparat ive example 2 | Inven tive steel B | 796 | 769 | 733 | 603 | 9.8 | 600 |
| | | | | | | | 700 |
| | | | | | | | 800 |
| | | | | | | | 900 |
| Inventiv e example 3 | Inven tive steel C | 792 | 775 | 740 | 410 | 11.8 | 600 |
| | | | | | | | 700 |
| | | | | | | | 800 |
| | | | | | | | 900 |
| Comparat ive example 3 | Compa rativ e steel D | 801 | 779 | 746 | 408 | 13.5 | 600 |
| | | | | | | | 700 |
| | | | | | | | 800 |
| | | | | | | | 900 |
| Comparat ive example 4 | Compa rativ e steel E | 795 | 776 | 742 | 411 | 12.5 | 600 |
| | | | | | | | 700 |
| | | | | | | | 800 |
| | | | | | | | 900 |
| Comparat ive example 5 | Compa rativ e steel F | 803 | 776 | 738 | 403 | 12.8 | 600 |
| | | | | | | | 700 |
| | | | | | | | 800 |
| | | | | | | | 900 |
| Comparat ive example 6 | Compa rativ e steel G | 795 | 768 | 734 | 411 | 11.6 | 600 |
| | | | | | | | 700 |
| | | | | | | | 800 |
| | | | | | | | 900 |

In Table 2, the unit of temperature is °C, the unit of the cooling rate is °C/sec., the FM start temperature refers to the non-recrystallization region rolling start temperature, and the FM end temperature refers to the non-recrystallization region rolling end temperature.

**[Table 3]**

| Classif ication | Steel type | Base material | | | | After linear heating | | | |
|---|---|---|---|---|---|---|---|---|---|
| | | Yiel d stre ngth | Tens ile stre ngth | Polyg onal ferri te (volu me %) | Impac t tough ness avera ge | Yield stren gth | Tens ile stre ngth | Individu Avera al ge impact impac toughnes t s tough ness | |
| Inventi ve example 1 | Inven tive steel A | 527 | 665 | 7.5 | 278 | 514 | 661 | 267/262/ 253 | 260 |
| | | | | | | 513 | 649 | 265/288/ 302 | 285 |
| | | | | | | 532 | 642 | 277/322/ 326 | 308 |
| | | | | | | 507 | 627 | 194/130/ 184 | 170 |
| Compara tive example 1 | Inven tive steel A | 525 | 654 | 24.5 | 79 | 509 | 646 | 45/56/12 8 | 76 |
| | | | | | | 502 | 635 | 79/65/84 | 76 |
| | | | | | | 500 | 624 | 56/102/2 8 | 62 |
| | | | | | | 498 | 612 | 57/58/38 | 51 |
| Inventi ve example 2 | Inven tive steel B | 538 | 672 | 6.7 | 247 | 534 | 668 | 245/167/ 158 | 190 |
| | | | | | | 529 | 659 | 264/286/ 302 | 284 |
| | | | | | | 518 | 642 | 268/231/ 188 | 229 |
| | | | | | | 510 | 621 | 154/186/ 109 | 150 |
| Compara tive example 2 | Inven tive steel B | 510 | 623 | 31.8 | 183 | 507 | 612 | 203/264/ 197 | 221 |
| | | | | | | 498 | 601 | 174/123/ 184 | 160 |
| | | | | | | 488 | 596 | 156/89/2 05 | 150 |
| | | | | | | 482 | 584 | 142/76/8 7 | 102 |
| Inventi ve example 3 | Inven tive steel C | 542 | 671 | 7.9 | 281 | 538 | 664 | 221/265/ 287 | 258 |
| | | | | | | 531 | 659 | 234/212/ 264 | 237 |
| | | | | | | 528 | 640 | 198/187/ 234 | 206 |
| | | | | | | 513 | 627 | 265/188/ 203 | 219 |
| Compara tive example 3 | Compa rativ e steel D | 587 | 689 | 22.1 | 134 | 567 | 678 | 75/68/32 | 58 |
| | | | | | | 552 | 670 | 15/78/54 | 49 |
| | | | | | | 542 | 652 | 103/28/3 6 | 56 |
| | | | | | | 523 | 641 | 28/64/28 | 40 |
| Compara tive example 4 | Compa rativ e steel E | 524 | 625 | 35.5 | 226 | 514 | 615 | 52/105/3 9 | 65 |
| | | | | | | 508 | 611 | 64/103/1 54 | 107 |
| | | | | | | 501 | 602 | 51/136/1 21 | 103 |
| | | | | | | 492 | 598 | 25/38/65 | 43 |
| Compara tive example 5 | Compa rativ e steel F | 536 | 628 | 38.4 | 193 | 523 | 613 | 156/123/ 158 | 146 |
| | | | | | | 512 | 607 | 126/154/ 130 | 137 |
| | | | | | | 503 | 598 | 78/123/1 62 | 121 |
| | | | | | | 494 | 588 | 58/28/42 | 43 |
| Compara tive example 6 | Compa rativ e steel G | 506 | 624 | 42 | 133 | 503 | 611 | 120/175/ 56 | 117 |
| | | | | | | 493 | 608 | 89/45/37 | 57 |
| | | | | | | 483 | 594 | 35/48/56 | 47 |
| | | | | | | 479 | 578 | 59/21/34 | 38 |

In Table 3, the unit of yield strength and tensile strength is MPa, and the unit of impact toughness is J.

When the mechanical properties of the base material and the mechanical properties after the linear heating are compared in Table 3, Inventive Examples 1 to 3, which all satisfied the alloy composition and manufacturing conditions according to the present invention, achieve the target yield strength, tensile strength and impact toughness at - 40°C.

Specifically, Inventive Examples 1 to 3 have the characteristics of yield strength of 500 MPa or greater, tensile strength of 600 MPa or greater, impact toughness of 100 J or greater at -40°C both before and after linear heating.

Comparative Example 3 uses comparative steel D in which the C content is excessive. It can be seen that strength is significantly higher than a target level but impact toughness is significantly reduced. This is considered to be due to formation of coarse carbide, which causes fracture in the impact test.

Comparative Example 4 uses comparative steel E in which the Mo component was insufficient and Comparative Example 5 uses comparative steel F in which the Nb component is insufficient. It can be seen that strength is remarkably reduced and impact toughness is lowered. This is because the amount of dissolved Mo and Nb is small and the amount of Mo and Nb is not sufficient to form a precipitate after linear heating. If Mo and Nb are added excessively, toughness may rather be deteriorated due to coarse precipitates, and thus, Mo and Nb must be added in the control range of the present invention.

Comparative Example 6 uses comparative steel G in which Mn and Ni components are insufficient. Since a sufficiently low Ar₃ temperature was not secured, a large amount of polygonal ferrite was formed during rolling at a low temperature, degrading strength and toughness.

Comparative Example 1 satisfied the alloy composition of the present invention, but the rolling temperature exceeded 850°C to lower impact toughness. Comparative Example 3 satisfied the alloy composition of the present invention, but the cooling conditions were out of the range of the present invention, resulting in an increase in a polygonal ferrite fraction to degrade strength and toughness due to the growth of crystal grain after linear heating.

While example exemplary embodiments have been shown and described above, it will be apparent to those skilled in the art that modifications and variations could be made without departing from the scope of the present invention as defined by the appended claims.

## Claims

1. A high-strength structural steel sheet having excellent heat treatment resistance, the high-strength structural steel sheet comprising:
by weight percent (wt%), 0.03 to 0.07% of C, 0.05 to 0.2% of Si, 1.6 to 2.3% of Mn, 0.008% or less of P, 0.002% or less of S, 0.025% or less of Al, 0.1 to 0.4% of Cu, 1.4 to 2.3% of Ni, 0.08 to 0.2% of Mo, 0.01 to 0.025% of Nb, 0.008 to 0.02% of Ti, 0.001 to 0.008% of N, the remainder being Fe, and unavoidable impurities,
wherein, by volume percent (vol%) a microstructure within 10 mm of the surface consists of 20% or less of polygonal ferrite and 80% or more of acicular ferrite, and
wherein the steel sheet has a yield strength of 500 MPa or greater, tensile strength of 600 MPa or greater, and impact toughness of 100 J or greater at -40°C.

2. The high-strength structural steel sheet of claim 1, wherein
a thickness of the steel sheet is 40 mm or less.

3. A method of manufacturing a high-strength structural steel sheet according to Claim 1 having excellent heat treatment resistance, the method comprising:
reheating a slab at 1100 to 1200°C wherein the slab includes, by weight percent (wt%), 0.03 to 0.07% of C, 0.05 to 0.2% of Si, 1.6 to 2.3% of Mn, 0.008% or less of P, 0.002% or less of S, 0.025% or less of Al, 0.1 to 0.4% of Cu, 1.4 to 2.3% of Ni, 0.08 to 0.2% of Mo, 0.01 to 0.025% of Nb, 0.008 to 0.02% of Ti, 0.001 to 0.008% of N, the remainder being Fe, and unavoidable impurities;
performing non-recrystallization region rolling on the reheated slab at 750 to 850°C; and
performing cooling to a cooling end temperature of 380 to 440°C at a cooling rate of 10°C/sec. or faster after the non-recrystallization region rolling, wherein the steel sheet has a yield strength of 500 MPa or greater, tensile strength of 600 MPa or greater, and impact toughness of 100 J or greater at-40°C.

4. The method of claim 3 , further comprising:
linearly heating the cooled steel sheet to 600 to 900°C and subsequently performing bending.

## Patentansprüche

1. Hochfestes Baustahlblech mit ausgezeichneter Wärmebehandlungsfestigkeit, wobei das hochfeste Baustahlblech umfasst:
nach Gewichtsprozent (Gew.-%), 0,03 bis 0,07 % C, 0,05 bis 0,2 % Si, 1,6 bis 2,3 % Mn, 0,008 % oder weniger P, 0,002 % oder weniger S, 0,025 % oder weniger Al, 0,1 bis 0,4 % Cu, 1,4 bis 2,3 % Ni, 0,08 bis 0,2 % Mo, 0,01 bis 0,025 % Nb, 0,008 bis 0,02 % Ti, 0,001 bis 0,008 % N, wobei der Rest Fe und unvermeidliche Verunreinigungen sind,
wobei, nach Volumenprozent (Vol.-%) eine Mikrostruktur innerhalb von 10 mm der Oberfläche aus 20 % oder weniger polygonalem Ferrit und 80 % oder mehr nadelförmigem Ferrit besteht, und
wobei das Stahlblech eine Fließfestigkeit von 500 MPa oder größer, Zugfestigkeit von 600 MPa oder größer und Schlagzähigkeit von 100 J oder größer bei -40 °C aufweist.

2. Hochfestes Baustahlblech nach Anspruch 1, wobei eine Dicke des Stahlblechs 40 mm oder weniger beträgt.

3. Verfahren zum Herstellen eines hochfesten Baustahlblechs nach Anspruch 1, welches ausgezeichnete Wärmebehandlungsfestigkeit aufweist, wobei das Verfahren umfasst:
Anlassen einer Tafel auf 1100 bis 1200 °C, wobei die Tafel beinhaltet, nach Gewichtsprozent (Gew.-%), 0,03 bis 0,07 % C, 0,05 bis 0,2 % Si, 1,6 bis 2,3 % Mn, 0,008 % oder weniger P, 0,002 % oder weniger S, 0,025 % oder weniger Al, 0,1 bis 0,4 % Cu, 1,4 bis 2,3 % Ni, 0,08 bis 0,2 % Mo, 0,01 bis 0,025 % Nb, 0,008 bis 0,02 % Ti, 0,001 bis 0,008 % N, wobei der Rest Fe und unvermeidliche Verunreinigungen sind;
Durchführen von nicht rekristallisierendem Bereichswalzen der angelassenen Tafel bei 750 bis 850 °C; und
Durchführen von Abkühlen bis zu einer Abkühltemperatur von 380 bis 440 °C bei einer Abkühlgeschwindigkeit von 10 °C/Sek. oder schneller nach dem nicht rekristallisierenden Bereichswalzen, wobei das Stahlblech eine Fließfestigkeit von 500 MPa oder größer, Zugfestigkeit von 600 MPa oder größer und Schlagzähigkeit von 100 J oder größer bei -40 °C aufweist.

4. Verfahren nach Anspruch 3, weiter umfassend:
lineares Erwärmen des abgekühlten Stahlblechs auf 600 bis 900 °C und darauf folgendes Biegen.

## Revendications

1. Tôle d'acier de construction à haute résistance présentant une excellente résistance au traitement thermique, la tôle d'acier de construction à haute résistance comprenant :
en pourcentage en poids (% en poids), 0,03 à 0,07 % de C, 0,05 à 0,2 % de Si, 1,6 à 2,3 % de Mn, 0,008 % ou moins de P, 0,002 % ou moins de S, 0,025 % ou moins d'Al, 0,1 à 0,4 % de Cu, 1,4 à 2,3 % de Ni, 0,08 à 0,2 % de Mo, 0,01 à 0,025 % de Nb, 0,008 à 0,02 % de Ti, 0,001 à 0,008 % de N, le reste étant du Fe, et des impuretés inévitables,
dans laquelle, en pourcentage en volume (% en volume), une microstructure à moins de 10 mm de la surface est constituée de 20 % ou moins de ferrite polygonale et de 80 % ou plus de ferrite aciculaire, et
dans laquelle la tôle d'acier a une limite d'élasticité de 500 MPa ou plus, une résistance à la traction de 600 MPa ou plus et une ténacité aux chocs de 100 J ou plus à -40 °C.

2. Tôle d'acier de construction à haute résistance selon la revendication 1,
dans laquelle l'épaisseur de la tôle d'acier est de 40 mm ou moins.

3. Procédé de fabrication d'une tôle d'acier de construction à haute résistance selon la revendication 1 ayant une excellente résistance au traitement thermique, le procédé comprenant :
le réchauffage d'une brame à une température de 1 100 à 1 200 °C, dans lequel la brame comporte, en pourcentage en poids (en poids %), 0,03 à 0,07 % de C, 0,05 à 0,2 % de Si, 1,6 à 2,3 % de Mn, 0,008 % ou moins de P, 0,002 % ou moins de S, 0,025 % ou moins d'Al, 0,1 à 0,4 % de Cu, 1,4 à 2,3 % de Ni, 0,08 à 0,2 % de Mo, 0,01 à 0,025 % de Nb, 0,008 à 0,02 % de Ti, 0,001 à 0,008 % de N, le reste étant du Fe, et des impuretés inévitables ;
l'exécution d'un laminage d'une région de non-recristallisation sur la brame réchauffée à une teméprature de 750 à 850 °C ; et
l'exécution d'un refroidissement jusqu'à une température finale de refroidissement de 380 à 440 °C à une vitesse de refroidissement de 10 °C/s ou plus rapidement après le laminage de la région de non-recristallisation, dans lequel la tôle d'acier a une limite d'élasticité de 500 MPa ou plus, une résistance à la traction de 600 MPa ou plus et une ténacité aux chocs de 100 J ou plus à -40 °C.

4. Procédé selon la revendication 3, comprenant en outre : le chauffage linéaire de la tôle d'acier refroidie à une température de 600 à 900 °C et l'exécution par la suite d'un pliage.
